



US006074454A

**United States Patent** [19]**Abrams et al.****Patent Number:** **6,074,454****Date of Patent:** **Jun. 13, 2000**[54] **LEAD-FREE FRANGIBLE BULLETS AND PROCESS FOR MAKING SAME**[75] Inventors: **John T. Abrams**, Raleigh; **Anil V. Nadkarni**, Chapel Hill, both of N.C.; **Roy Kelly**, Arlington, Va.[73] Assignee: **Delta Frangible Ammunition, LLC**, Stafford, Va.[21] Appl. No.: **08/678,776**[22] Filed: **Jul. 11, 1996**[51] **Int. Cl.**<sup>7</sup> **F42B 8/14; F42B 12/74; C22C 1/04; C22C 1/09**[52] **U.S. Cl.** **75/247; 75/231; 75/232; 75/233; 75/235; 75/236; 75/237; 75/238; 75/244; 75/252; 75/254; 102/506; 102/517; 102/529; 419/2; 419/28; 419/29; 419/38; 419/47; 419/56; 419/58; 419/59**[58] **Field of Search** **75/231-233, 235-238, 75/244, 247, 252, 254; 419/2, 29, 38, 47, 28, 56, 58, 59; 102/444, 459, 506, 514, 517, 448, 529**[56] **References Cited**

## U.S. PATENT DOCUMENTS

|           |         |                |          |
|-----------|---------|----------------|----------|
| 2,409,307 | 10/1946 | Patch et al.   | 102/92.5 |
| 2,995,090 | 8/1961  | Daubenspeck    | 102/91   |
| 3,123,003 | 3/1964  | Lange, Jr.     | 102/91   |
| 4,005,660 | 2/1977  | Pichard        | 102/92.1 |
| 4,165,692 | 8/1979  | Dufort et al.  | 102/92.7 |
| 4,881,465 | 11/1989 | Hooper et al.  | 102/501  |
| 4,949,645 | 8/1990  | Hayward et al. | 102/517  |

|           |         |                         |          |
|-----------|---------|-------------------------|----------|
| 5,069,869 | 12/1991 | Nicolas et al.          | 419/28   |
| 5,078,054 | 1/1992  | Sankaranarayanan et al. | 102/517  |
| 5,237,930 | 8/1993  | Belanger et al.         | 102/529  |
| 5,279,787 | 1/1994  | Oltrogge                | 419/38   |
| 5,399,187 | 3/1995  | Mravic et al.           | 75/228   |
| 5,442,989 | 8/1995  | Anderson et al.         | 86/20.12 |
| 5,527,376 | 6/1996  | Amick et al.            | 75/246   |
| 5,616,642 | 4/1997  | West et al.             | 524/439  |

## FOREIGN PATENT DOCUMENTS

|           |         |                |         |
|-----------|---------|----------------|---------|
| 531389    | 1/1941  | United Kingdom | .       |
| 2 278423A | 11/1994 | United Kingdom | 102/515 |

## OTHER PUBLICATIONS

ASM Handbook, vol. 7, Powder Metallurgy pp. 798-801, 121-122, 710-716, 802-813, 1984.

Condensed Chemical Dictionary, Tenth Ed., 1981, pp. 147, 1981.

Primary Examiner—Daniel J. Jenkins

Attorney, Agent, or Firm—Kalow Springut &amp; Bressler LLP

[57] **ABSTRACT**

The invention relates to bullets having increased frangibility (or which can be easily fragmented) and to materials and processes for the manufacture of such bullets. The bullets of the present invention are typically made from copper or copper alloy powders (including brass, bronze and dispersion strengthened copper) which are pressed and then sintered under conditions so as to obtain bullets with the desired level of frangibility. In preferred embodiments of the invention, the bullets also contain several additives that increase or decrease their frangibility.

**66 Claims, 3 Drawing Sheets****9 MM BULLET - NOMINAL DIMENSIONS**



9 MM BULLET - NOMINAL DIMENSIONS

**FIGURE 1**



.40 CALIBER BULLET - NOMINAL DIMENSIONS

## FIGURE 2



FRANGIBLE BULLET TEST SETUP

**FIGURE 3**

## LEAD-FREE FRANGIBLE BULLETS AND PROCESS FOR MAKING SAME

### BACKGROUND OF THE INVENTION

Traditionally bullets for small arms ammunition have been manufactured from lead and lead alloys. The major advantages of lead as a bullet material are its relatively low cost, high density and high ductility. The high density of lead has been particularly important to bullet design because the energy generated by the weight of a bullet is critical to the proper functioning of modern semi-automatic and automatic weapons, the in-flight stability of the round, and the terminal effects of the bullet.

The highly toxic nature of lead, however, and its propensity to fume and generate airborne particulate, place the shooter at an extreme health risk. The more a range is used, the more lead residue builds up, and the greater the resulting lead fume and lead dust pollution (particularly for indoor ranges). Moreover, the lead bullet residue left in the earthen berm of outdoor ranges can leach into the soil and contaminate water tables. In order for indoor ranges to operate safely, they require extensive and expensive air filtration systems, and both indoor and outdoor ranges require constant de-leading. These clean up operations are time consuming, costly and repetitive. Accordingly, there is a great need for lead-free bullets.

Additionally, personnel at range operations are concerned with the ricochet potential and the likelihood of causing "back-splatter" of the training ammunition. Back-splatter is a descriptive term for the bullet debris that bounces back in the direction of the shooter after a bullet impacts on a hard surface, such as steel targets or backstops. Ricochets present a significant hazard to individuals, equipment and structures in and around live firing ranges. A ricochet can be caused by a glancing impact by a bullet on almost any medium. Back-splatter presents a significant danger to shooters, training personnel standing on or around the firing line and observers. When a bullet strikes a hard surface at or near right angles, the bullet will either break apart or deform. There is still energy in the bullet mass, however, and that mass and its energy must go somewhere. Since the target material or backstop is impenetrable, the mass bounces back in the direction of the shooter.

It is believed that a key way to minimizing the risk of both ricochet and back-splatter is to maximize the frangibility of the bullet. By designing the bullet to fracture into small pieces, one reduces the mass of each fragment, in turn reducing the overall destructive energy remaining in the fragments.

Several prior art patents disclose materials and methods for making non-toxic or frangible bullets or projectiles. For example, U.S. Pat. No. 5,442,989 to Anderson discloses projectiles wherein the casing is frangible and made out of molded stainless steel powder or a stainless steel+pure iron powder mix with up to 2% by weight of graphite. The casing encloses a penetrator rod made of a hard material such as tungsten or tungsten carbide. This projectile is mainly for 20-35 mm cannons to engage targets such as armored vehicles, trucks, buildings, ships, etc. Upon impact against the target, the casing produces fragments which are thrown in all directions with great energy while the penetrator rod pierces the target.

U.S. Pat. No. 4,165,692 to Dufort discloses a projectile with a brittle sintered metal casing having a hollow interior chamber defined by a tapering helix with sharp edge stress risers which provide fault lines and cause the projectile to

break up into fragments upon impact against a hard surface. The casing is made of pressed iron powder which is then sintered. This projectile is also designed for large caliber rounds such as 20 mm cannon shots.

U.S. Pat. No. 5,399,187 to Mravic et. al. discloses a lead-free bullet which comprises sintered composite having one or more high density powders selected from tungsten, tungsten carbide, ferrotungsten, etc., and a lower density constituent selected from tin, zinc, iron, copper or a plastic matrix material. These composite powders are pressed and sintered. The high density constituent allows bullet densities approaching 9 g/cm<sup>3</sup>.

U.S. Pat. No. 5,078,054 to Sankaranarayanan et. al. discloses a frangible projectile comprising a body formed from iron powder with 2 to 5% by weight of graphite or iron with 3 to 7% by weight of Al<sub>2</sub>O<sub>3</sub>. The powders are compacted by cold pressing in a die or isostatic pressing, and then sintered.

U.S. Pat. No. 5,237,930 to Belanger et. al. discloses a frangible practice ammunition comprising compacted mixture of fine copper powder and a thermoplastic resin selected from nylon 11 and nylon 12. The copper content is up to about 93% by weight. The bullets are made by injection molding and are limited to densities of about 5.7 g/cm<sup>3</sup>. A typical 9 mm bullet only weighs about 85 grains.

None of the above discussed patents disclose or suggest lead-free, frangible bullets made of predominately copper with densities approaching that of conventional bullets. An objective of this invention is to provide a range of lead-free frangible bullets, optimized for frangibility, which will eliminate the lead fumes and dust hazard to the shooter while also minimizing the ricochet and back-splatter hazards. A further objective is to provide a low cost material and process for making such a bullet. Yet another objective is to provide a bullet with a weight (hence density) as high and as close to the conventional lead bullet as possible so that the recoil and the firing characteristics closely resemble those of conventional lead bullets. Yet another objective is to reduce the risk of lead residues leaching into the soil and water table in and around shooting ranges.

### SUMMARY OF THE INVENTION

The invention relates to bullets having increased frangibility (or which can be easily fragmented) and to powder materials and processes for the manufacture of such bullets. The bullets of the present invention are made from copper or copper alloy powders, including brass, bronze and dispersion strengthened copper. In preferred embodiments of the invention, the bullets also contain several additives that increase or decrease their frangibility. Additionally, the invention provides a simple low cost process to make bullets that is amenable to mass production via automation.

### BRIEF DESCRIPTION OF THE DRAWINGS

FIG. 1—shows a side elevation view of a typical 9 mm bullet.

FIG. 2—shows a side elevation view of a typical 40 caliber bullet.

FIG. 3—shows a frangible bullet test setup.

### DETAILED DESCRIPTION OF THE PREFERRED EMBODIMENTS

The embodiments described in this section and illustrated in the drawings are intended as examples only and are not to be construed as limiting. In fact there are hundreds of bullet

designs (at least) that could be made using the materials and the processes described in this disclosure. Moreover, the present disclosure is not intended as a treatise on bullet manufacturing and readers are referred to appropriate, available texts in the field for additional and detailed information on bullet manufacture and other aspects of practicing the invention.

Referring to FIGS. 1 and 2, typical bullets have a cylindrical body (1) with a tapered nose portion (2). The tip of the nose (3) can have various shapes, e.g., it can be flat as shown in FIG. 2, radiused as in FIG. 1 or spherical for better aerodynamics. The base (4) can be flat or have a boat tail on it or be in other shapes.

Copper is the preferred material of choice for making the bullets of this invention. It is non-toxic and has a reasonably high density—8.96 g/cm<sup>3</sup> vs. 11.3 g/cm<sup>3</sup> for lead. Copper powder technologies offer ways to make the bullets frangible; the metal is otherwise very ductile and will deform excessively and ricochet upon impact against a hard surface. The preferred process to make the bullets of this invention involves first blending the powder with a suitable lubricant, typically a stearate or wax, and then cold compacting the powder in a die at a pressure that produces a part having a green strength sufficient to permit handling of the part without chipping. The density of the compacted part is adjusted to provide sufficient interconnected porosity to allow for the lubricant vapor to escape during subsequent sintering treatment.

The bullets are then preferably sintered by heating in a protective atmosphere to prevent oxidation. The sintering can be done in a belt furnace which has three zones. The first zone called the “preheat zone” is set to a temperature sufficient to burn the lubricant off, typically 1000–1200° F. The second zone called the “high heat” zone is set to the sintering temperature, typically the 1500–1900° F. range, the exact temperature depending on the material and the frangibility required. The third zone called the “cool zone” typically has a water jacket surrounding it which allows the bullets to be cooled to room temperature in a protective atmosphere. The sintering time is adjusted by controlling the belt speed. The bullets may be repressed or coined after the sintering treatment to increase their density further. This allows production of heavier bullets by using a longer preform and yet keeping the overall dimensions of the final bullets the same. Optionally, the bullets may be resintered if necessary to provide higher ductility or reduced frangibility.

Copper powder pressed to a density between 7.5 to 8.5 g/cm<sup>3</sup>, preferably about 8.0 g/cm<sup>3</sup> and sintered at 1500 to 1900° F., preferably about 1700° F., has been found to have excellent firing characteristics and frangibility. Lower density and lower sintering temperature increase the frangibility while higher density and higher sintering temperature increase the ductility. A delicate balance must be struck between frangibility and ductility. The bullets must have sufficient ductility to withstand the firing operation without breaking up in the barrel of the gun or in flight up to the target. The bullet must also have sufficient frangibility so that it breaks up into small pieces upon impact against a hard surface.

It must be noted that different users of ammunition may prefer different degrees of frangibility. Some prefer to have complete breakup into powder to eliminate any ricochet or back-splatter and minimum penetration of the steel backstop while others will require retention of base pieces sufficiently large to preserve the rifling marks to assist in identifying the weapon which fired the bullet. Some others may prefer

breakup into small pieces rather than powder to minimize airborne particles, and at the same time also minimize the ricochet potential.

The technology disclosed in this invention can accommodate most, if not all, of the frangibility requirements. As mentioned above, one way to control frangibility is through control of density, sintering temperature and sintering time. Another way is to use additives to the copper powder. Several elements or compounds can be added to the copper powder to increase or decrease frangibility and reduce penetration of and damage to range backstops. One of the objects of these additives is to coat the copper powder particles with inert second phases and thus partially impede the sintering process so that the bonds formed between the particles are embrittled. One group of additives are oxides such as Al<sub>2</sub>O<sub>3</sub>, SiO<sub>2</sub>, TiO<sub>2</sub>, MgO, MoO<sub>3</sub>, etc. These may be added in powder form and blended or mechanically milled with the copper powder, or chemically formed by processes such as internal oxidation. One particular embodiment of this invention is to use a commercial Al<sub>2</sub>O<sub>3</sub> Dispersion Strengthened Copper (DSC) produced by the internal oxidation process. As the examples will show, the DSC material and copper with mixed SiO<sub>2</sub> powder produced bullets with excellent firing characteristics and increased frangibility. Surprisingly, MoO<sub>3</sub> addition decreased frangibility.

Another group of additives is solid lubricants such as graphite, MoS<sub>2</sub>, MnS, CaF<sub>2</sub>, etc. As the examples will show, the bullets made using graphite as an additive showed good firing characteristics and increased frangibility, while MoS<sub>2</sub> addition decreased frangibility.

Yet another group of additives is nitrides such as BN, SiN, AlN, etc. Boron nitride in hexagonal crystallographic form (HBN) is preferred as this behaves much like graphite and acts as a solid lubricant. Bullets made with HBN as an additive have good firing characteristics and increased frangibility.

The additives mentioned above can be used in combinations as well. For example, bullets made with graphite and SiO<sub>2</sub> additions show good firing characteristics and increased frangibility.

Additionally, carbides such as WC, SiC, TiC, NbC, etc., and borides such as TiB<sub>2</sub>, ZrB<sub>2</sub>, CaB<sub>6</sub> may also be used to increase the frangibility.

Common copper alloy powders such as brass and bronze can also be used to make the bullets of this invention. These alloys are harder than copper and thus need to be pressed at higher pressures. Lower sintering temperatures must be used for these alloys, as brass loses zinc by vaporization while the bronze produces lower melting phases. Recommended sintering temperatures for the bullets of this invention are 1500 to 1700° F. Some of the additives described above for copper can also be used for brass and bronze powders if necessary to increase the frangibility. Mixtures of copper and zinc or copper and tin powders may also be used instead of prealloyed brass and bronze powders.

## EXAMPLES

The following examples illustrate embodiments of the process and the lead-free frangible bullets of the present invention.

### Example I

Five different grades of copper powder produced by SCM Metal Products, Inc. (hereinafter “SCM”) were blended with a lubricant. These were assigned following blend numbers:

- 1) 99.75% 150RXM+0.25% Acrawax®C
- 2) 99.75% 150RXH **30** 0.25% Acrawax®C
- 3) 99.75% 100RXM+0.25% Acrawax®C
- 4) 99.75% 100RXH+0.25% Acrawax®C
- 5) 99.75% FOS-WC+0.25% Acrawax®C

Acrawax® is a trademark of Lonza Corporation. The generic name for Acrawax® is N,N'-ethylenebisstearamide, and its chemical family is alkyl amide. RXM, RXG, FOS-WS are grade designations of copper powder manufactured by SCM Metal Products, Inc. AL-25 is the grade designation for a dispersion strength copper material. Its generic designation in the Unified Number System (UNS) is C15725. Glid Cop® is the trademark for this material and is owned by SCM Metal Products, Inc.

About 115 grain (7.5 g) samples of the powder blend were pressed (molded) in a die to make the 9 mm bullets shown in FIG.-1. The bullets were sintered in a belt furnace under nitrogen. Density of bullets was determined using the water immersion technique.

The sintered bullets were loaded by Delta Frangible Ammunition LLC (hereinafter "Delta") into 9 mm Luger® primed cartridge cases using sufficient commercial smokeless propellant to produce velocities and pressures within the range normally encountered for 9 mm Luger® ammunition. The completed rounds were test fired. The test setup is shown in FIG.-3. Both instrumented test barrels and commercially available 9 mm pistols and sub-machine guns (**5**) were used. The absence of breakup in the barrel or in flight was determined by placing paper witness cards (**6**) along the flight of the bullet. Frangibility was determined by allowing the bullets to impact a thick (5/8 inch) steel backstop (**7**) placed perpendicular to the bullet's line of flight at the rear end of a wooden collection box (**8**). The bullets entered the collection box through a hole covered with a paper witness card. The fragments generated from the impact of the bullets against the steel plate were collected. Any intact "bases" were pulled out and the rest of the fragments were screened over a Tyler 14 mesh (1190  $\mu\text{m}$ ) screen. The component collected over the screen ( $>1190 \mu\text{m}$ ) was labeled "chunks" and the remainder passing through the screen ( $<1190 \mu\text{m}$ ) was labeled "powder". Each component was weighed and the weight percentage of each was calculated as a percentage of the total mass collected. In order to rate the different compositions of the invention as to their frangibility, weight factors were assigned to the three components as follows:

Powder: 60% or 0.60

Chunks: 30% or 0.30

Bases: 10% or 0.10

The "score" for each composition was calculated by multiplying the weight % of each component by its weight factor and adding the three numbers as follows:

$$\text{Score} = 0.60 \times \text{Wt. \% Powder} + 0.30 \times \text{Wt. \% Chunks} + 0.10 \times \text{Wt. \% Bases}$$

Frangibility ratings were then developed based on the score for each composition as follows:

| Score | Frangibility Rating |
|-------|---------------------|
| <15   | 1                   |
| 16-25 | 2                   |
| 26-35 | 3                   |
| 36-45 | 4                   |
| >45   | 5                   |

The rating of 1, representing the lowest frangibility, had the highest weight % of bases while the rating of 5, representing the highest frangibility, had the highest weight % of powder.

Table-1 shows the pertinent processing data on the bullets and the firing test results. The data shows that densities over 8.2 g/cm<sup>3</sup> were achieved; this compares to 5.7 g/cm<sup>3</sup> typical of commercial injection molded copper-nylon bullets of the type described in U.S. Pat. No. 5,237,930 (the disclosure of which is incorporated by reference into the present disclosure). The higher densities allow heavier bullets to be produced without changing the overall dimensions; in fact it is possible to produce 120 grain bullets in the geometry shown in FIG.-1 which compares to 80-85 grain bullets typical of the copper-nylon type described above. These bullets thus more closely resemble the firing characteristics of conventional lead bullets now used in the field.

None of the bullets broke up in the gun barrel or flight, indicating good integrity. The data in Table 1 shows that the bullets made from the above copper powders had satisfactory frangibility. The 150RXH grade of copper had higher frangibility than the other grades examined. All these bullets did very little damage to the steel backstop.

## Example II

This example illustrates the effect of oxide additions on frangibility. Copper powder grade 150RXM was used as the control material and all results were compared to the bullets made from this powder. Additions of oxides were made to this powder to determine their effects. In one experiment the FOS-WC copper powder was used. GlidCop® dispersion strengthened copper AL-25 (copper+0.5 wt. % Al<sub>2</sub>O<sub>3</sub>) grade powder produced by SCM was also used in one of the experiments. The following powder blends were made:

- 6) 99.70% 150RXM+0.05% SiO<sub>2</sub>+0.25% Acrawax®C
- 7) 99.65% 150RXM+0.10% SiO<sub>2</sub>+0.25% Acrawax®C
- 8) 99.65% 150RXM+0.10% MoO<sub>3</sub>+0.25% Acrawax®C
- 9) 99.50% FOS-WC+0.25% SiO<sub>2</sub>+0.25% Acrawax®C
- 10) 99.75% AL-25+0.25% Acrawax C

Bullets were produced and test fired as described in Example I.

Table 2 shows the relevant processing and firing test data. The data shows that addition of SiO<sub>2</sub> does indeed increase frangibility. Blend 7 containing 0.10% SiO<sub>2</sub> made significantly more frangible bullets than the comparable Blend 1, while the addition of 0.05% SiO<sub>2</sub> in Blend 6 did not appear to have a significant effect on frangibility. The addition of 0.25% SiO<sub>2</sub> in Blend 9 coupled with the lower compaction pressure (lower density) and lower sintering temperature, on the other hand, made the bullet too frangible and it broke up before hitting the target. A higher compaction pressure (higher density) and higher sintering temperature may produce a bullet with sufficient integrity to survive firing. GlidCop® AL-25 which contains 0.5% Al<sub>2</sub>O<sub>3</sub> (Blend 10) also made a bullet that survived the firing and broke up when it hit the target. This bullet was not as frangible as the control bullets of Blend 1, but this is believed to be due to the high sintering temperature normally used for GlidCop®. The frangibility of GlidCop® bullet could be increased further by reducing the sintering temperature or lowering the density. Surprisingly, the addition of MoO<sub>3</sub> (Blend 8) decreased the frangibility significantly; there was almost no powder recovered in the fragments. It is possible that the high partial pressure generated at sintering temperature by the dissociation of MoO<sub>3</sub> could have aided in the vapor transport of copper atoms, thus activating the sintering process and creating stronger more ductile bonds.

## Example III

This example illustrates the effect of solid lubricants on frangibility. Graphite and MoS<sub>2</sub> were used as solid lubricants. Following blends were made:

- 11) 99.70% 150RXM+0.05% graphite+0.25% Acrawax C  
 12) 99.65% 150RXM+0.10% graphite+0.25% Acrawax C  
 13) 99.50% FOS-WC+0.25% graphite+0.25% Acrawax C  
 14) 99.65% 150RXM+0.10% MoS<sub>2</sub>+0.25% Acrawax C  
 Bullets were produced and test fired as described in Example I.

Table 3 shows the relevant processing and firing test data. The data shows that 0.05% graphite (Blend 11) does not change the frangibility, while 0.10% graphite (Blend 12) increases frangibility somewhat, as indicated by the higher score for this material. However, a higher amount of graphite is needed to increase frangibility significantly. Addition of 0.25% graphite to FOS-WC copper in Blend 13 made the bullet so frangible it broke up in the barrel, although this may have been due to the lower density and lower sintering temperature used. Higher density and higher sintering temperature would most likely produce a bullet with sufficient ductility to withstand firing. The addition of 0.10% MoS<sub>2</sub> (Blend 14) had the same surprising effect as observed with MoO<sub>3</sub> in that the frangibility decreased significantly. Here again, some effect of the additive on the sintering kinetics of copper is suspected.

#### Example IV

This example illustrates the effect of combined addition of an oxide and a solid lubricant. Blends were made with two different levels of SiO<sub>2</sub> and graphite added to the 150RXM powder. A blend was also made with graphite addition to AL-25 as follows:

- 15) 99.70% 150RXM+0.025% SiO<sub>2</sub>+0.025% graphite+0.25% Acrawax C  
 16) 99.65% 150RXM+0.05% SiO<sub>2</sub>+0.05% graphite+0.25% Acrawax C  
 17) 99.50% AL-25+0.25% graphite+0.25% Acrawax C

Bullets were made and test fired as described in Example I.

Table 4 shows the relevant processing and firing test data. The data shows that a combined addition of graphite and SiO<sub>2</sub> had an effect similar to the addition of either of the components at the same level. A level of 0.05% (Blend 15) did not have a significant effect on the frangibility while a level of 0.10% (Blend 16) did have a significant effect. Addition of 0.25 graphite to GlidCop® AL-25 (Blend 17) made a bullet with sufficient ductility to survive firing, but significantly higher frangibility than plain AL-25 as in Blend 10.

#### Example V

This example illustrates the effect of a nitride addition on frangibility. A blend was made with an addition of hexagonal boron nitride (HBN) as follows:

- 18) 99.65% 150RXM+0.10% HBN+0.25% Acrawax C  
 Bullets were produced and test fired as described in Example I.

Table 5 shows the relevant processing and test firing data. HBN is not only a nitride, it has a crystallographic structure identical to graphite in that the hexagonal platelets slide over each other readily. Therefore, it is used as a solid lubricant. The frangibility data shows that an HBN addition had the same effect to that of graphite at the same level. At 0.10% addition (Blend 18), the frangibility was increased somewhat, but higher additions would be required to make a more significant impact on frangibility. Other nitrides including the cubic form of boron nitride (CBN) could also be used although the latter may be too abrasive to the 10  
 15  
 20  
 25  
 30  
 35  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990  
 5995  
 6000  
 6005  
 6010  
 6015  
 6020  
 6025  
 6030  
 6035  
 6040  
 6045  
 6050  
 6055  
 6060  
 6065  
 6070  
 6075  
 6080  
 6085  
 6090  
 6095  
 6100  
 6105  
 6110  
 6115  
 6120  
 6125  
 6130  
 6135  
 6140  
 6145  
 6150  
 6155  
 6160  
 6165  
 6170  
 6175  
 6180  
 6185  
 6190  
 6195  
 6200  
 6205  
 6210  
 6215  
 6220  
 6225  
 6230  
 6235  
 6240  
 6245  
 6250  
 6255  
 6260  
 6265  
 6270  
 6275  
 6280  
 6285  
 6290  
 6295  
 6300  
 6305  
 6310  
 6315  
 6320  
 6325  
 6

TABLE 1-continued

| 9 mm Bullet Processing and Test Results |                |                   |                        |           |           |                        |                        |              |                     |
|-----------------------------------------|----------------|-------------------|------------------------|-----------|-----------|------------------------|------------------------|--------------|---------------------|
| Blend No.                               | Pressure (ksi) | Mold Temp. (° F.) | Sinter Density (g/cm³) | Breakup   |           | Powder <1190 µm (wt %) | Chunks >1190 µm (wt %) | Bases (wt %) | Frang. Score Rating |
|                                         |                |                   |                        | in Barrel | or Flight |                        |                        |              |                     |
| 4                                       | 80             | 1700              | 8.20                   | No        |           | 9.5                    | 28.4                   | 62.1         | 20 2                |
| 5                                       | 68             | 1500              | 8.02                   | No        |           | 5.4                    | 23.3                   | 71.3         | 17 2                |

TABLE 2

| 9 mm Bullet Processing and Test Results |                |                   |                        |           |           |                        |                        |              |                     |
|-----------------------------------------|----------------|-------------------|------------------------|-----------|-----------|------------------------|------------------------|--------------|---------------------|
| Blend No.                               | Pressure (ksi) | Mold Temp. (° F.) | Sinter Density (g/cm³) | Breakup   |           | Powder <1190 µm (wt %) | Chunks >1190 µm (wt %) | Bases (wt %) | Frang. Score Rating |
|                                         |                |                   |                        | in Barrel | or Flight |                        |                        |              |                     |
| 6                                       | 80             | 1700              | 8.23                   | No        |           | 10.4                   | 20.2                   | 69.4         | 19 2                |
| 7                                       | 80             | 1700              | 8.23                   | No        |           | 14.1                   | 50.7                   | 35.1         | 27 3                |
| 8                                       | 80             | 1700              | 8.27                   | No        |           | 0.4                    | 18.2                   | 81.4         | 14 1                |
| 9                                       | 68             | 1500              | 7.92                   | Yes       |           | 59.6                   | 29.8                   | 10.6         | 46 5                |
| 10                                      | 64             | 1860              | 8.30                   | No        |           | 5.4                    | 33.6                   | 61.0         | 19 2                |

TABLE 3

| 9 mm Bullet Processing and Test Results |                |                   |                        |           |           |                        |                        |              |                     |
|-----------------------------------------|----------------|-------------------|------------------------|-----------|-----------|------------------------|------------------------|--------------|---------------------|
| Blend No.                               | Pressure (ksi) | Mold Temp. (° F.) | Sinter Density (g/cm³) | Breakup   |           | Powder <1190 µm (wt %) | Chunks >1190 µm (wt %) | Bases (wt %) | Frang. Score Rating |
|                                         |                |                   |                        | in Barrel | or Flight |                        |                        |              |                     |
| 11                                      | 80             | 1700              | 8.25                   | No        |           | 8.7                    | 19.5                   | 71.8         | 18 2                |
| 12                                      | 80             | 1700              | 8.23                   | No        |           | 11.0                   | 38.7                   | 50.3         | 23 2                |
| 13                                      | 64             | 1500              | 8.02                   | Yes       |           | 53.4                   | 34.4                   | 12.2         | 44 4                |
| 14                                      | 80             | 1700              | 8.40                   | No        |           | 0.8                    | 20.5                   | 78.7         | 14 1                |

TABLE 4

| 9 mm Bullet Processing and Test Results |                |                   |                        |           |           |                        |                        |              |                     |
|-----------------------------------------|----------------|-------------------|------------------------|-----------|-----------|------------------------|------------------------|--------------|---------------------|
| Blend No.                               | Pressure (ksi) | Mold Temp. (° F.) | Sinter Density (g/cm³) | Breakup   |           | Powder <1190 µm (wt %) | Chunks >1190 µm (wt %) | Bases (wt %) | Frang. Score Rating |
|                                         |                |                   |                        | in Barrel | or Flight |                        |                        |              |                     |
| 15                                      | 80             | 1700              | 8.26                   | No        |           | 12                     | 21                     | 67           | 20 2                |
| 16                                      | 80             | 1700              | 8.20                   | No        |           | 15                     | 53                     | 32           | 28 3                |
| 17                                      | 64             | 1860              | 8.28                   | No        |           | 8.7                    | 74.2                   | 17.0         | 29 3                |

TABLE 5

| 9 mm Bullet Processing and Test Results |                |                   |                        |           |           |                        |                        |              |                     |
|-----------------------------------------|----------------|-------------------|------------------------|-----------|-----------|------------------------|------------------------|--------------|---------------------|
| Blend No.                               | Pressure (ksi) | Mold Temp. (° F.) | Sinter Density (g/cm³) | Breakup   |           | Powder <1190 µm (wt %) | Chunks >1190 µm (wt %) | Bases (wt %) | Frang. Score Rating |
|                                         |                |                   |                        | in Barrel | or Flight |                        |                        |              |                     |
| 18                                      | 80             | 1700              | 8.21                   | No        |           | 18                     | 30                     | 52           | 20 2                |

TABLE 6

| 9 mm Bullet Processing and Test Results |                     |                     |                 |                             |                        |                        |              |       |               |  |
|-----------------------------------------|---------------------|---------------------|-----------------|-----------------------------|------------------------|------------------------|--------------|-------|---------------|--|
| Blend No.                               | Mold Pressure (ksi) | Sinter Temp. (° F.) | Density (g/cm³) | Breakup in Barrel or Flight | Powder <1190 µm (wt %) | Chunks >1190 µm (wt %) | Bases (wt %) | Score | Frang. Rating |  |
| 19A                                     | 88                  | 1500                | 7.68            | Yes                         | 79                     | 21                     | 0            | 54    | 5             |  |
| 19B                                     | 96                  | 1606                | 7.76            | Yes                         | 26                     | 69                     | 5            | 37    | 4             |  |
| 19C                                     | 88                  | 1700                | 7.88            | No                          | 2                      | 60                     | 38           | 23    | 2             |  |
| 20A                                     | 88                  | 1500                | 8.24            | Yes                         | 80                     | 20                     | 0            | 54    | 5             |  |
| 20B                                     | 88                  | 1600                | 8.32            | No                          | 0                      | 27                     | 73           | 16    | 1             |  |

What is claimed is:

1. A frangible bullet comprising at least 60 percent by weight copper and manufactured by pressing a copper-containing powder in a die to form a pressed powder compact and subsequently sintering said pressed powder compact, wherein said sintering is partially impeded either
    - (i) by the addition of a frangibility effecting additive to said powder, or
    - (ii) through control of density of said pressed powder compact, or
    - (iii) through control of sintering temperature, or sintering time, or
 any combination of the above; so as to produce a bullet capable of fragmenting upon impact with a target.
  2. The bullet of claim 1 wherein the bullet is lead-free.
  3. The bullet of claim 1 wherein the powder is a dispersion strengthened copper powder.
  4. The bullet of claim 3 wherein the dispersion strengthened copper powder is made by internal oxidation of a dilute solid solution alloy of copper and a reactive element selected from the group consisting of Si, Al, Ti, and Mg.
  5. Ammunition comprising the bullet of claim 1.
  6. The bullet of claim 1, wherein the sintering is partially impeded by addition of a frangibility effecting additive to said powder; said additive being selected from the group consisting of an oxide, a solid lubricant, a nitride, a carbide, a boride, and a combination of any thereof.
  7. The bullet of claim 1 wherein the sintering is partially impeded either
    - (i) through control of density of said pressed powder compact, or
    - (ii) through control of sintering temperature, or sintering time, or any combination thereof.
  8. The bullet of claim 7, wherein the powder is a dispersion strengthened copper powder.
  9. The bullet of claim 8 wherein the dispersion strengthened copper powder is made by internal oxidation of a dilute solid solution alloy of copper and a reactive element selected from the group consisting of Si, Al, Ti, and Mg.
  10. The bullet of claim 7, wherein the powder is a prealloyed brass containing from 5 to 40 percent by weight of zinc.
  11. The bullet of claim 7, wherein the powder is a mixture of copper powder and from 5 to 40 percent by weight of zinc powder.
  12. The bullet of claim 7 wherein the powder is a prealloyed bronze containing from 2 to 20 percent by weight of tin.
  13. The bullet of claim 7 wherein the powder is a mixture of copper powder and from 2 to 20 percent by weight of tin powder.
  14. The bullet of claim 7, wherein the powder comprises at least about 99.5 percent by weight copper.
- 15      15. The bullet of claim 7, wherein the powder is a mixture of about 90 percent by weight copper and about 10 percent by weight tin.
16. The bullet of claim 7, wherein the powder is a mixture of about 70 percent by weight copper and about 30 percent by weight zinc.
- 20      17. The bullet of claim 7, wherein the powder is a prealloyed bronze containing 10 percent by weight tin.
18. The bullet of claim 7, wherein the powder is a prealloyed brass containing 30 percent by weight zinc.
- 25      19. The bullet of claim 6 wherein the frangibility effecting additive comprises an oxide additive.
- 20      20. The bullet of claim 19 wherein the oxide additive is selected from the group consisting of  $\text{SiO}_2$ ,  $\text{Al}_2\text{O}_3$ ,  $\text{TiO}_2$ ,  $\text{MgO}$ ,  $\text{MoO}_3$  and combinations thereof.
- 30      21. The bullet of claim 20 wherein the oxide additive is  $\text{SiO}_2$ ,  $\text{Al}_2\text{O}_3$ ,  $\text{TiO}_2$ ,  $\text{MgO}$  or a combination thereof and the amount of oxide additive is from 0.05 to 1.0 percent by weight.
22. The bullet of claim 20 wherein the powder comprises from 0.05 to 0.50 percent by weight of  $\text{MoO}_3$ .
- 35      23. The bullet of claim 6 wherein the frangibility effecting additive comprises a solid lubricant additive.
24. The bullet of claim 23 wherein the solid lubricant additive is selected from the group consisting of graphite,  $\text{MoS}_2$ ,  $\text{MnS}$ ,  $\text{CaF}_2$  and combinations thereof.
- 40      25. The bullet of claim 24 wherein the solid lubricant additive is graphite,  $\text{MnS}$ ,  $\text{CaF}_2$  or a combination thereof and the amount of solid lubricant additive is from 0.05 to 1.0 percent by weight.
26. The bullet of claim 24 wherein the powder comprises from 0.05 to 0.50 percent by weight of  $\text{MoS}_2$ .
- 45      27. The bullet of claim 6 wherein the frangibility effecting additive comprises a nitride additive.
28. The bullet of claim 27 wherein the nitride additive is selected from the group consisting of HBN,  $\text{SiN}$ ,  $\text{AlN}$  and combinations thereof and the amount of nitride additive is from 0.05 to 1.0 percent by weight.
- 50      29. The bullet of claim 6 wherein the frangibility effecting additive comprises an oxide additive and a solid lubricant additive.
30. The bullet of claim 29 wherein the oxide additive is selected from the group consisting of  $\text{SiO}_2$ ,  $\text{Al}_2\text{O}_3$ ,  $\text{TiO}_2$ , and  $\text{MgO}$  and the solid lubricant additive is selected from the group consisting of graphite,  $\text{MnS}$ , and  $\text{CaF}_2$  and the combined amount of oxide and solid lubricant additives is from 0.05 to 1.0 percent by weight.
- 55      31. The bullet of claim 6 wherein the frangibility effecting additive comprises a carbide additive.
32. The bullet of claim 31 wherein the carbide additive is selected from the group consisting of WC,  $\text{SiC}$ ,  $\text{TiC}$ ,  $\text{NbC}$  and combinations thereof and the amount of carbide additive is from 0.05 to 1.0 percent by weight.
- 60      33. The bullet of claim 6 wherein the frangibility effecting additive comprises a boride additive.

**34.** The bullet of claim **33** wherein the boride additive is selected from the group consisting of  $TiB_2$ ,  $ZrB_2$ ,  $CaB_6$  and combinations thereof and the amount of boride additive is from 0.05 to 1.0 percent by weight.

**35.** The bullet of claim **6** wherein the powder is a prealloyed brass containing from 5 to 40 percent by weight of zinc.

**36.** The bullet of claim **6** wherein the powder is a mixture of copper powder and from 5 to 40 percent by weight of zinc powder.

**37.** The bullet of claim **6** wherein the powder is a prealloyed bronze containing from 2 to 20 percent by weight of tin.

**38.** The bullet of claim **6** wherein the powder is a mixture of copper powder and from 2 to 20 percent by weight of tin.

**39.** A method of making a frangible bullet which comprises pressing a powder containing at least 60 percent by weight copper in a die to form a pressed powder compact and subsequently sintering said pressed powder compact, wherein said sintering is partially impeded either

(i) by the addition of a frangibility effecting additive to said powder, or

(ii) through control of density of said pressed powder compact, or

(iii) through control of sintering temperature, or sintering time, or

any combination of the above; so as to produce a bullet capable of fragmenting upon impact with a target.

**40.** The method of claim **39**, wherein the sintering is partially impeded either

(ii) through control of density of said pressed powder compact, or

(iii) through control of sintering temperature, or sintering time, or any combination thereof.

**41.** The method of claim **40** wherein the pressing of the powder is performed at a pressure ranging from 50 to 120 ksi.

**42.** The method of claim **41** wherein the pressing is done at a pressure ranging from 60 to 100 ksi.

**43.** The method of claim **40** wherein the sintering is performed in a protective atmosphere at a temperature ranging from about 1500 to about 1900° F. for a length of time ranging from about 10 to about 120 minutes.

**44.** The method of claim **43** wherein the sintering is done at a temperature of 1600 to 1800° F. when the powder is copper, between 1600 and 1700° F. when the powder is brass and between 1500 and 1600° F. when the powder is bronze.

**45.** The method of claim **43** wherein the protective atmosphere is nitrogen or a mixture of nitrogen and hydrogen or reaction products of a combusted hydrocarbon.

**46.** The method of claim **43** wherein the sintering time is between 15 and 45 minutes.

**47.** The method of claim **43** wherein the bullet is repressed after the sintering step.

**48.** The method of claim **47** wherein the bullet is resin-tered after repressing.

**49.** A powder useful for manufacturing a frangible item by pressing in a die and subsequently sintering, said powder comprising at least about 60 percent by weight copper and a frangibility effecting additive selected from the group consisting of an oxide, a solid lubricant, a nitride, a carbide, a boride, and combinations thereof.

**50.** A powder of claim **49**, wherein the amount of the additive is from 0.05 to 1.0 percent by weight of the powder.

**51.** A powder of claim **49**, wherein the additive is an oxide selected from the group consisting of  $SiO_2$ ,  $Al_2O_3$ ,  $TiO_2$ ,  $MgO$ ,  $MoO_3$ , and combinations thereof.

**52.** A powder of claim **51**, wherein the amount of the oxide additive is from 0.05 to 1.0 percent by weight of the powder.

**53.** A powder of claim **49**, wherein the additive is a solid lubricant selected from the group consisting of graphite,  $MoS_2$ ,  $MnS$ ,  $CaF_2$ , and combinations thereof.

**54.** A powder of claim **53**, wherein the amount of the solid lubricant additive is from 0.05 to 1.0 percent by weight of the powder.

**55.** A powder of claim **49**, wherein the additive is a nitride selected from the group consisting of  $HBN$ ,  $SiN$ ,  $AlN$ , and combinations thereof.

**56.** A powder of claim **35**, wherein the amount of the nitride additive is from 0.05 to 1.0 percent by weight of the powder.

**57.** A powder of claim **35**, wherein the additive is a carbide selected from the group consisting of  $WC$ ,  $SiC$ ,  $TiC$ ,  $NbC$ , and combinations thereof.

**58.** A powder of claim **57**, wherein the amount of the carbide additive is from 0.05 to 1.0 percent by weight of the powder.

**59.** A powder of claim **49**, wherein the additive is a boride selected from the group consisting of  $TiB_2$ ,  $ZrB_2$ ,  $CaB_6$ , and combinations thereof.

**60.** A powder of claim **59**, wherein the amount of the boride additive is from 0.05 to 1.0 percent by weight of the powder.

**61.** A powder of claim **49**, wherein the additive is a combination of an oxide and a solid lubricant.

**62.** A powder of claim **61**, wherein the oxide additive is selected from the group consisting of  $SiO_2$ ,  $Al_2O_3$ ,  $TiO_2$  and  $MgO$  and the solid additive is selected from the group consisting of graphite,  $MnS$ , and  $CaF_2$  and the combined amount of the oxide and solid lubricant additives is from 0.05 to 1.0 percent by weight.

**63.** A powder of claim **49**, wherein the powder further contains from 5 to 40 percent by weight of zinc powder.

**64.** A powder of claim **49**, wherein the powder further contains from 2 to 20 percent by weight of tin powder.

**65.** A powder of claim **49**, wherein the powder comprises a copper alloy comprised of from 5 to 40 percent by weight of zinc.

**66.** A powder of claim **49**, wherein the powder comprises a copper alloy comprised of from 2 to 20 percent by weight of tin.



US006074454C1

(12) EX PARTE REEXAMINATION CERTIFICATE (8897th)  
**United States Patent**  
**Abrams et al.**

(10) Number: **US 6,074,454 C1**  
(45) Certificate Issued: **Mar. 13, 2012**

(54) **LEAD-FREE FRANGIBLE BULLETS AND PROCESS FOR MAKING SAME**

(75) Inventors: **John T. Abrams**, Raleigh, NC (US);  
**Anil V. Nadkarni**, Chapel Hill, NC (US); **Roy Kelly**, Arlington, VA (US)

(73) Assignee: **Delta Frangible Ammunition, LLC**,  
New York, NY (US)

**Reexamination Request:**  
No. 90/009,288, Sep. 29, 2008

**Reexamination Certificate for:**

Patent No.: **6,074,454**  
Issued: **Jun. 13, 2000**  
Appl. No.: **08/678,776**  
Filed: **Jul. 11, 1996**

(51) **Int. Cl.**

**F42B 12/00** (2006.01)  
**F42B 12/074** (2006.01)  
**C22C 1/004** (2006.01)  
**C22C 32/00** (2006.01)

(52) **U.S. Cl.** ..... **75/247**; 102/506; 102/517;  
102/529; 419/28; 419/38; 419/56; 419/47;  
419/59; 419/58; 419/29; 419/2; 75/238;  
75/237; 75/236; 75/235; 75/233; 75/232;  
75/231; 75/254; 75/252; 75/244

(58) **Field of Classification Search** ..... None  
See application file for complete search history.

(56) **References Cited**

To view the complete listing of prior art documents cited during the proceeding for Reexamination Control Number 90/009,288, please refer to the USPTO's public Patent Application Information Retrieval (PAIR) system under the Display References tab.

*Primary Examiner*—Jerry D. Johnson

(57) **ABSTRACT**

The invention relates to bullets having increased frangibility (or which can be easily fragmented) and to materials and processes for the manufacture of such bullets. The bullets of the present invention are typically made from copper or copper alloy powders (including brass, bronze and dispersion strengthened copper) which are pressed and then sintered under conditions so as to obtain bullets with the desired level of frangibility. In preferred embodiments of the invention, the bullets also contain several additives that increase or decrease their frangibility.



**9 MM BULLET - NOMINAL DIMENSIONS**

**1**

**EX PARTE  
REEXAMINATION CERTIFICATE  
ISSUED UNDER 35 U.S.C. 307**

THE PATENT IS HEREBY AMENDED AS  
INDICATED BELOW.

**2**

AS A RESULT OF REEXAMINATION, IT HAS BEEN  
DETERMINED THAT:

Claims 1, 2, 5-7, 12-15, 23, 24, 38-42, 49, 50, 53, 54, 64  
and 66 are cancelled.

<sup>5</sup> Claims 3, 4, 8-11, 16-22, 25-37, 43-48, 51, 52, 55-63 and  
65 were not reexamined.

\* \* \* \* \*